

## UNITED STATES PATENT OFFICE.

JEAN F. P. DE LA RIBOISIERE, OF WASHINGTON, DISTRICT OF COLUMBIA.

## FUEL FOR INTERNAL-COMBUSTION ENGINES.

No Drawing.

Application filed November 18, 1924. Serial No. 750,657.

*To all whom it may concern:*

Be it known that I, JEAN F. P. DE LA RIBOISIERE, a citizen of the French Republic, residing at Washington, D. C., U. S. A., have invented certain new and useful Improvements in Fuel for Internal-Combustion Engines, of which the following is a specification.

This invention relates to improvements in fuels for internal combustion engines, of the character disclosed in my application for Patent Serial No. 664586, filed September 24, 1923, of which the present application is a continuation in part. In said application I have described an engine fuel including liquid hydrocarbons boiling above 160° C., combined with an ether and a phenolic body. As stated in said application I have discovered that a large proportion of liquid hydrocarbons boiling above 160° C. may be utilized in low boiling point fuels, such as benzol, benzine or gasoline, providing the liquid hydrocarbons boiling above 160° C. are combined with an ether to promote the combustion or ignition of the mixture, and a phenolic body to retain the ether in the mixture.

The primary object of the present invention is to improve fuels of this type by employing a body containing a phenyl radical. Among the compounds that I have found satisfactory are the phenyl compounds of selenium, tellurium, thorium, thallium, uranium, tungsten, titanium, bismuth, vanadium, aluminum, etc. These metallic phenyl compounds may be used but, of course, my invention is not limited to the use of these specific metallic phenyl compounds, as others may be used. While I prefer to use metallic phenyl compounds because they are more stable, my invention is not limited thereto. Other compounds containing the phenyl radical may be used in connection with the other ingredients of my fuel composition. For example, dibenzyl salicylate, the benzyl amines, the benzyl anilines, the benzyl alcohols and their derivatives may be used. The benzyl-hydroxy amines may also be used.

I have found from actual practice, that a mixture of this character will increase the speed of many types of motor vehicles at least 20 percent when climbing a steep hill. A demonstration in connection with a num-

ber of different types of motor cars shows an increase of speed in climbing a steep hill of from 20 to 30 percent. As a matter of fact, in using fuel of this character, it has been demonstrated that the present mixture will increase the power of the motor at least 25 percent, and effect an economy in the consumption of fuel of about 30 percent over a similar demonstration with ordinary gasoline.

In practical use it has been found that phenyl compounds, when radio active, have a very great influence on the power efficiency of the motor.

As examples of fuel mixtures which I have found to give very good results, I state as follows:

|                                                                   | Per cent. |
|-------------------------------------------------------------------|-----------|
| 1. Low boiling point hydrocarbons<br>(such as gasoline or benzol) | 68        |
| High boiling point hydrocarbons<br>(such as heavy gas oil)        | 30        |
| Ether                                                             | 1.5       |
| Phenyl compound, for example di-phenyl telluride                  | 0.5       |
| 2. Low boiling point hydrocarbons                                 | 58        |
| High boiling point hydrocarbons<br>(such as kerosene)             | 80        |
| Ether                                                             | 2.5       |
| Phenyl compound, for example di-phenyl telluride                  | 2.5       |
| 3. Low boiling point hydrocarbons<br>(including benzol)           | 30        |
| High boiling point hydrocarbons                                   | 40        |
| Alcohol                                                           | 27        |
| Ether                                                             | 1.5       |
| Phenyl compound, for example di-phenyl telluride                  | 1.5       |
| 4. Low boiling point hydrocarbons                                 | 30        |
| High boiling point hydrocarbons<br>(such as kerosene)             | 57        |
| Ether                                                             | 3         |
| Phenyl compounds                                                  | 10        |
| 5. Low boiling point hydrocarbons<br>(such as gasoline or benzol) | 68        |
| High boiling point hydrocarbons<br>(such as gas oil)              | 30        |
| Ether                                                             | 1.6       |
| Dibenzyl diselenide                                               | .4        |
| 6. Low boiling point hydrocarbons                                 | 60        |
| High boiling point hydrocarbons<br>(such as kerosene)             | 37        |
| Ether                                                             | 2.5       |
| Triphenyl of thallium                                             | 1         |

|                                                                    | Per cent. |
|--------------------------------------------------------------------|-----------|
| 7. Low boiling point hydrocarbons                                  | 60        |
| High boiling point hydrocarbons<br>(such as kerosene)              | 37        |
| 5. Ether                                                           | .5        |
| Tetra phenyl of uranium                                            | 2.5       |
| 8. Low boiling point hydrocarbons                                  | 60        |
| High boiling point hydrocarbons<br>(such as kerosene)              | 35.5      |
| 10. Ether                                                          | .5        |
| Tetra phenyl of vanadium, or other<br>phenyl compounds of vanadium | 4         |
| 9. Low boiling point hydrocarbons                                  | 60        |
| High boiling point hydrocarbons<br>(such as kerosene)              | 32        |
| 15. Ether                                                          | 1         |
| Dibenzyl salicylate                                                | 7         |
| 10. Low boiling point hydrocarbons                                 | 60        |
| High boiling point hydrocarbons<br>(such as kerosene)              | 37.5      |
| 20. Ether                                                          | .5        |
| Benzyl aniline                                                     | 2         |
| 11. Low boiling point hydrocarbons                                 | 60        |
| High boiling point hydrocarbons                                    | 36.5      |
| 25. Ether                                                          | .5        |
| Benzyl hydroxylamine                                               | 3         |

While I have disclosed a few preferred examples, it is obvious that these proportions may be varied to suit conditions.

What I claim and desire to secure by Letters Patent is:

1. An improved fuel for internal combustion engines including liquid hydrocarbons boiling above 160° C., and a smaller proportion of an ether and a compound containing a non-hydroxy phenyl radical.
2. An improved fuel for internal combus-

tion engines including a proportion of liquid hydrocarbons boiling above 160° C., a small proportion of ether adapted to promote the combustion or ignition thereof, and a proportion of non-hydroxy phenyl compounds.

3. An improved fuel for internal combustion engines including a considerable proportion of liquid hydrocarbons boiling above 160° C., a small proportion of an ether adapted to promote the combustion or ignition thereof, and a proportion of metallic phenyl compounds.

4. An improved fuel for internal combustion engines including liquid hydrocarbons boiling above 160° C., and a smaller proportion of an ether and radioactive metallic phenyl compounds.

5. An improved fuel for internal combustion engines including a proportion of liquid hydrocarbons boiling above 160° C., a small proportion of ether adapted to promote the combustion or ignition thereof, and a proportion of radioactive metallic phenyl compounds.

6. An improved fuel for internal combustion engines including liquid hydrocarbons boiling above 160° C., and a smaller proportion of an ether and a phenyl compound of a metal.

7. An improved fuel for internal combustion engines including liquid hydrocarbons boiling above 160° C., and a smaller proportion of an ether and a nonhydroxy phenyl compound.

In testimony whereof I hereunto affix my signature.

JEAN F. P. DE LA RIBOISIERE.